

Aug. 27, 1968

W. J. BRENNAN

3,399,093

METHOD AND APPARATUS FOR THE MANUFACTURE OF  
VULCANIZED FIBER SHEET MATERIALS

Filed June 23, 1965



INVENTOR.  
WILLIAM J. BRENNAN

BY

*Thomas J. Dugan*

ATTORNEY

## 1

3,399,093

**METHOD AND APPARATUS FOR THE MANUFACTURE OF VULCANIZED FIBER SHEET MATERIALS**

William J. Brennan, Bridgeport, Pa., assignor to The Budd Company, Philadelphia, Pa., a corporation of Pennsylvania

Filed June 23, 1965, Ser. No. 466,311  
5 Claims. (Cl. 156—76)**ABSTRACT OF THE DISCLOSURE**

A pair of rollers is provided to receive a vulcanized fiber sheet material therebetween. One of the rollers is heated and the other is cooled. The material is kept under tension as it leaves the rollers.

This invention relates to an improved method and apparatus for the manufacture of vulcanized fiber sheet materials. More particularly it concerns a novel apparatus and method for calendering relatively thin vulcanized fiber sheet materials to remove and eliminate undulations of portions of the material.

The term "vulcanized fiber" referred to herein denotes a tough, horny cellulosic material. Vulcanized fiber is made by treating substantially cellulosic fibrous materials with a hydrolyzing agent. The most commonly used hydrolyzing agent is zinc chloride. The hydrolyzing agent gelatinizes the surfaces of the cellulosic fibers and the individual fibers adhere to each other. When the hydrolyzing agent is leached from the cellulosic fibers, strong bonds develop between the individual fibers, and a tough, dense material is obtained.

The term "bagginess" as used herein denotes a condition that occurs in sheet materials in which portions of the sheet become undulated or corrugated. A sheet of baggy fiber has an overall appearance of being warped and somewhat wrinkled.

Vulcanized fiber is a relatively old material. It was the forerunner of many of today's modern plastics. Bagginess has been a constant problem confronting vulcanized fiber producers since vulcanized fiber was first introduced almost a century ago. Bagginess makes it difficult, if not impossible, to process the vulcanized fiber sheets in fabricating operations.

It has heretofore been proposed to form the vulcanized fiber under relatively high tension in an attempt to pull out the bagginess. However, it was found that the use of the higher tensions aggravated the baggy condition. It was heretofore proposed to use virtually no tension in the manufacture of vulcanized fiber. This was also unsuccessful. Various combinations of high tension and low tension, and variations in drying conditions were attempted to correct the problem of bagginess. None of the methods suggested proved satisfactory.

Accordingly, it is the object of this invention to provide an improved method and apparatus to produce flat vulcanized fiber sheet material.

It is another object of this invention to provide a method whereby undulations and corrugations of vulcanized fiber sheets can be removed and eliminated.

It is another object of this invention to provide apparatus to remove and eliminate bagginess from vulcanized fiber.

It is a further object of this invention to provide an apparatus and method to produce substantially flat vulcanized fiber sheet materials.

It is a further object of this invention to provide a method and apparatus that with a minimum change of present operating procedures will eliminate bagginess of vulcanized fiber sheet materials.

## 2

The other objects and advantages of the present invention will become apparent from the hereinafter detailed description and the appended claims when read in conjunction with the accompanying drawings in which:

5 FIG. 1 is a pictorial illustration of a sheet of baggy vulcanized fiber.

FIG. 2 is a schematic representation of an apparatus for the continuous formation of relatively thin vulcanized fiber sheet materials.

10 FIG. 3 is an enlarged illustration of the calender and wind-up reel as shown in the apparatus of FIG. 2.

FIG. 4 is an illustration of an alternative embodiment of the apparatus of FIG. 3 having air convection means.

15 FIG. 5 is an alternative embodiment of the apparatus as illustrated in FIG. 3 having a cooling chamber.

It is to be understood that the forms of the invention herewithin shown and described are to be taken as preferred embodiments. In describing the preferred embodiments of the invention illustrated in the drawings, specific terminology will be resorted to for the sake of clarity. However, it is not intended to be limited to the specific terms so selected, and it is to be understood that each specific term includes all technical equivalents which operate in a similar manner to accomplish a similar purpose.

Turning now to the drawings, the number 10 designates the sheet of baggy vulcanized fiber of FIG. 1. The edges 12 of the sheet and the center portions 14 are undulated. 30 Because of the undulations, the baggy fiber sheet material will not lie flat in punching operations, and cannot be coated uniformly. Relatively thin vulcanized fiber sheet materials are especially susceptible to becoming baggy.

35 The relatively thin vulcanized fiber sheets, that is sheets .005 to .125 inch thick, may be manufactured in a continuous process utilizing the system of FIG. 2. In this process a ply, or plurality of plies 16, of substantially cellulosic paper are fed through a concentrated zinc chloride solution 18. The zinc chloride is absorbed by the paper. Excess zinc chloride is removed by a set of nip rolls 20. The zinc chloride is permitted to react on the cellulose in a reaction zone 22.

40 After a controlled amount of reaction has taken place, the zinc chloride is removed from the plies in a series of steps in leaching tanks 24. The percent of the zinc chloride in the vulcanizing fiber is gradually reduced until in the final tank 30 the vulcanized fiber contains substantially no zinc chloride.

45 The vulcanized fiber can then be dried in an oven 33 where it is supported by a conveyor belt. The vulcanized fiber can then be further dried by passing it over a set of can dryers 32. The moisture content of the fiber is generally reduced to an amount above 4%, but below 55 10%. The vulcanized fiber is then passed through calender 34 and reeled up for shipment.

50 The vulcanized fiber is advanced through the processing equipment by tension of one type or another. The plies when wet are easily stretched and deformed, especially in the early stages of vulcanization. Non-uniform stretching of the sheet is believed to cause a portion of the bagginess.

55 In the vulcanization process, the plies shrink in both the machine direction and the cross machine direction. This shrinkage produces a complex combination of internal stresses in the vulcanized fiber.

60 Vulcanized fiber exhibits limited thermoplastic properties when it contains moisture and is relatively warm. For the vulcanized fiber to be thermoplastic, it must contain at least 4% moisture by weight and be at a temperature above 120° F. The thermoplastic properties of vulcanized fiber increase with increases in temperature. In com-

mercial practice it has been found that the temperature of the fiber should be maintained substantially above 120° F. and preferably in the range of 180°-200° F. in order to obtain the maximum utility of the thermoplastic property.

In the prior art processes the vulcanized fiber was dried to a moisture content above 4% and was packed relatively hot. Temperatures of the fiber as packed were often in excess of 160° F.

When the vulcanized fiber was packed, it exhibited a limited amount of bagginess. After remaining in storage for a week or so, the fiber became extremely baggy. This was due to the aforementioned internal stresses distorting the warm, moist thermoplastic vulcanized fiber.

It was initially believed that either reducing the moisture content or cooling the vulcanized fiber would prevent bagginess. This was an erroneous assumption. The bagginess that occurred in the vulcanization process was sufficiently great to impair the utility of the final product. Neither reducing the moisture content or cooling the fiber reduced this bagginess. It was found that it was not practical to reduce the moisture content sufficiently low to prevent bagginess because the fiber became brittle and quickly regained moisture from the atmosphere.

Accordingly, what was required was a method and apparatus to remove the bagginess that developed during vulcanization and to control the stresses in the vulcanized fiber to prevent further development of bagginess. This is obtained according to the teachings of this invention by initially raising and maintaining the temperature of the vulcanized fiber above 120° F., and preferably between 160°-200° F. while simultaneously forming the sheet into a flat configuration. This initial step removes the bagginess that is formed as a result of the vulcanization process. The heated flat vulcanized fiber is maintained in a flat configuration while it is cooled preferably below 120 degrees F. This second step sets or removes the internal stresses and prevents development of bagginess in storage.

An apparatus especially well suited to perform the above steps is illustrated in FIG. 3. The calendar stack 34 has a first roll 38 mounted in pressure contact with a second roll 40. Both the first and second rolls 38 and 40 are substantially right cylinders. The rolls may have a certain amount of crown to correct bowing. Both rolls 38 and 40 are rigid and have surfaces that are free of undulations. The rolls provide flat surfaces against which the vulcanized fiber may be formed into a flat sheet. The rolls 38 and 40 are mounted to rotate on their axes. The rolls may be either free moving or driven.

The first roll 38 is heated. The roll may be heated by introducing and circulating in the interior of the roll a heated fluid medium, for example, superheated steam or a high temperature liquid. The temperature to which the roll is maintained is dependent on certain factors. The primary function of the heated roll is to raise and maintain temperature of the vulcanized fiber to between 120° F. and 200° F. The factors which dictate how high the temperature of the first roll 38 must be maintained are the initial temperature of the fiber, the temperature to which the vulcanized fiber is to be heated, and the length of time that the fiber is in contact with the first roll. In most applications the temperature of the first roll should be maintained at approximately 250° to 270°.

The second roll 40 is cooled. The roll 40 may be cooled by introducing and circulating a cooling fluid medium within the interior of the roll. A primary function of the second roll 40 is to act as a heat exchanger removing heat from the vulcanized fiber sheet. The temperature of the vulcanized fiber sheet should be reduced substantially. The temperature should be reduced at least twenty degrees, and preferably to a temperature below 120° F. Accordingly, the coolant must maintain the roll at a relatively low temperature. It has been found that in most applications the coolant must be maintained at a temperature

approximately 0° F. to reduce the temperature of the fiber to an acceptable range.

In operation, a sheet of vulcanized fiber containing at least 4% moisture is passed about a substantial portion of the periphery of the first roll 38. While in contact with the roll 38, the temperature of the sheet is raised to and maintained at a first temperature above 120° F. At this first temperature condition and the moisture condition as noted, the sheet becomes plastic and conforms to the configuration of the surface of roll 38. The bagginess which is a result of the vulcanization process is thereby removed.

The vulcanized fiber sheet is then passed about a major portion of the periphery of the second roll 40. The temperature of the vulcanized fiber sheet is reduced while in contact with the surface of the second roll 40. The fiber is set in a flat configuration by cooling it while in contact with the surface of the second roll 40. The temperature of the fiber should be reduced at least 20 degrees below the first temperature and preferably to below 120° F. The take-up reel 36 provides sufficient tension to hold the vulcanized fiber sheet in contact with both rolls 38 and 40 during the heating and cooling steps.

The most difficult step is cooling the vulcanized fiber. If the apparatus of FIG. 3 is utilized, substantially all of the cooling must be done by the second roll 40. The rate of production is somewhat limited by this factor.

An alternative embodiment of the apparatus of this invention is illustrated in FIG. 4. In addition to the calendar stack 34 of the embodiment of FIG. 3, means 44 to convect air about the vulcanized fiber sheet are provided. In the illustration, fans 44 are shown. This apparatus has several advantages over the apparatus of FIG. 3.

The vulcanized fiber sheet is held in a flat configuration and under a tension between the contact point of the first and second rolls 38 and 40, and the take-up reel 36. By circulating cooling air about the fiber at this point, as illustrated in FIG. 4, it is possible to remove the heat from the vulcanized fiber sheet quickly and efficiently. Using the apparatus of FIG. 4, the optimum results obtainable with the apparatus of FIG. 3 are achieved with increased speed and efficiency of operation.

In situations where it is not possible or practical to use the air convection means as shown in FIG. 4, an apparatus as shown in FIG. 5 may be utilized. This apparatus is similar to the apparatus of FIG. 3, but contains in addition to the calendar a cooling chamber 46.

The cooling chamber may be utilized to reduce the temperature of the vulcanized fiber sheet in a manner similar to the aforementioned convection means. The vulcanized fiber sheet is held in a taut, flat condition as it passes through the chamber 46. The fiber is set in this flat condition. The cooling chamber 46 is not as desirable as the convection apparatus of FIG. 4 in that the cooling chambers are more expensive to purchase and more difficult to maintain and use.

It is to be understood that the forms of the invention herewithin shown and described are to be taken as preferred embodiments. Various changes may be made in the apparatus without departing from the scope or spirit of the invention. For example, calendar stacks having more than two rolls may be used. In addition, combinations of stacks may be used in which one stack is heated and one stack cooled. These, and other similar embodiments, are within the scope of this invention.

Having thus described my invention, I claim:

1. A calendering apparatus for .005 to .125 inch thick vulcanized fiber sheet materials capable of removing and impairing formation of bagginess in said material, the apparatus comprising in combination: means for feeding a plurality of plies of substantially cellulosic paper through a concentrated zinc chloride solution whereby said zinc chloride is absorbed by said paper to react therewith to form vulcanized fiber sheet material, means including

leaching tanks for removing said zinc chloride from said material, means for drying said material to reduce the moisture content below 10% but greater than 4%, at least two rigid, temperature controllable, calender rolls, said rolls being substantially right cylinders and being mounted to rotate about their axes and in pressure contact; means advancing said material about a major portion of the peripheral surfaces and through the contact point of said rolls; means introducing and circulating a heated fluid medium within the interior of a first of said rolls and heating maintaining the temperature of the material while in contact with the surface of said first roll at a first temperature above 120° F.; means introducing and circulating a cooling fluid medium within the interior of a second of said rolls; reducing and maintaining the temperature of said material substantially below the said first temperature; means rotating the rolls in a heat exchange relationship with respect to said vulcanized fiber sheet material; and means for maintaining said vulcanized fiber sheet material under tension while it is in contact with said rolls.

2. An improved apparatus for continuous manufacture of .005 to .125 inch thick vulcanized fiber sheet material comprising means for feeding a plurality of plies of substantially cellulosic paper through a concentrated zinc chloride solution whereby said zinc chloride is absorbed by said paper to react therewith to form vulcanized fiber sheet material, means including leaching tanks for removing said zinc chloride from said material, means for drying said material to reduce the moisture content below 10% but greater than 4%; a calendering apparatus adapted to remove and impair formation of bagginess of the vulcanized fiber sheet material, said apparatus comprising in combination: at least two, rigid, hollow, substantially right cylindrical rolls, said rolls being mounted to rotate about their axes and in pressure contact; means causing said material to advance about a substantial portion of the periphery and between the contact points of said rolls; means introducing and circulating a heating fluid medium within interior of a first of said rolls raising and maintaining the temperature of the material contacting the surface of the said first roll at a first temperature above 120° F.; means introducing and circulating a cooling fluid medium within the interior of a second of said rolls to reduce the temperature of the material contacting the surface of the said second roll substantially below the said first temperature; means rotating the rolls about their axes in a heat exchange relationship with respect to said vulcanized fiber sheet material; and means for maintaining said sheet material under tension while it is in contact with said rolls.

3. A method for removing and impairing formation of bagginess in vulcanized fiber sheet materials which comprises the ordered steps of: passing a plurality of plies of substantially cellulosic paper through a concentrated zinc chloride solution to cause said zinc chloride to be absorbed by said paper to react therewith to form a sheet of vulcanized fiber, removing said zinc chloride from said

sheet, drying said sheet to a point not less than 4% moisture by weight, advancing said sheet of vulcanized fiber containing least 4% moisture by weight over a substantial portion of the peripheral surface of a first, rigid, right cylindrical roll, simultaneously heating and maintaining the sheet at a temperature above 120° F., conforming said sheet to the configuration of said first roll; compressing said sheet between said first roll and a second, rigid, right cylindrical roll; and advancing said sheet over a substantial portion of the peripheral surface of said second roll, simultaneously reducing the temperature substantially below the said first temperature; and maintaining said sheet under tension when it is between said first and second rolls.

4. A method for removing and impairing formation of bagginess in vulcanized fiber sheet materials which comprises the ordered steps of: passing a plurality of plies of substantially cellulosic paper through a concentrated zinc chloride solution to cause said zinc chloride to be absorbed by said paper to react therewith to form a sheet of vulcanized fiber, removing said zinc chloride from said sheet, drying said sheet to a point not less than 4% moisture by weight, advancing said sheet of vulcanized fiber containing at least 4% moisture by weight over a substantial portion of the peripheral surface of the first, rigid, right cylindrical roll, simultaneously heating and maintaining the sheet at a temperature above 120° F. conforming the said sheet to the configuration of said first roll; compressing said sheet between said first roll and a second, rigid, right cylindrical roll; advancing said sheet over a substantial portion of the peripheral surface of said second roll, simultaneously reducing the temperature to a second temperature substantially below said first temperature; and circulating cooling air about said sheet, reducing said temperature of said sheet below said second temperature; and maintaining said sheet under tension when it is between said first and second rolls.

5. The method of claim 3 wherein the said first temperature is above 160° F. and below 200° F.

40

#### References Cited

##### UNITED STATES PATENTS

|           |         |             |       |         |
|-----------|---------|-------------|-------|---------|
| 2,385,916 | 10/1945 | Hahn        | ----- | 118—69  |
| 3,189,515 | 6/1965  | Phillips    | ----- | 161—269 |
| 2,251,890 | 8/1941  | Montgomery  | ----- | 162—206 |
| 2,318,111 | 4/1943  | Steinberger | ----- | 264—284 |
| 2,551,005 | 4/1951  | Johnson     | ----- | 264—284 |
| 2,631,954 | 3/1953  | Bright      | ----- | 264—175 |
| 3,004,296 | 10/1961 | Snedecker   | ----- | 264—175 |

##### FOREIGN PATENTS

|         |         |         |
|---------|---------|---------|
| 484,560 | 7/1952  | Canada. |
| 586,366 | 11/1959 | Canada. |
| 659,880 | 3/1963  | Canada. |

EARL M. BERGERT, Primary Examiner.

M. L. KATZ, Assistant Examiner.